

May 19, 1970

K. BROTHZMANN ET AL

3,512,957

STEELMAKING PROCESSES

Filed June 19, 1964

4 Sheets-Sheet 1

*Fig. 1*



*Fig. 2*



May 19, 1970

K. BROTZMANN ET AL

3,512,957

STEELMAKING PROCESSES

Filed June 19, 1964

4 Sheets-Sheet 2



May 19, 1970

K. BROTZMANN ET AL

3,512,957

STEELMAKING PROCESSES

Filed June 19, 1964

4 Sheets-Sheet 3

*Fig. 4*



May 19, 1970

K. BROTMANN ET AL

3,512,957

STEELMAKING PROCESSES

Filed June 19, 1964

4 Sheets-Sheet 4

*Fig. 5*



## 1

3,512,957  
STEELMAKING PROCESSES

Karl Brotzmann, Westhofen-Buchholz, near Schwerte (Ruhr), Germany, and Eric R. Morgan, Pittsburgh, Pa., assignors to Dortmund-Hörder Huttenunion Aktiengesellschaft, Dortmund, Germany

Filed June 19, 1964, Ser. No. 376,420

Claims priority, application Germany, Aug. 10, 1963,

D 42,212

Int. Cl. C21c 7/06, 7/10, 33/00

U.S. Cl. 75—49

7 Claims

To make deep-drawing steels resistant to aging, the steel is de-oxidised with aluminum leaving at least 0.025% of Al dissolved in the steel. Some of the aluminum oxide forming as a de-oxidation product is deposited as large oxide particles near the surface of the ingot on casting, so that the entire ingot must be flame-descaled. Apart from the cost of this descaling, production is greatly reduced as a result. Also, small oxide particles are still left beneath the ingot surface and as a result the Al-killed steel cannot be used for purposes requiring best surface qualities. On the other hand, the cold working properties of the steel are so superior to those of non-ageing-resistant steel that a considerable amount of deep-drawing sheets are produced in this way.

There has been no lack of attempts so to alter the steel structure as to obviate the considerable difficulties occurring during its manufacture. For example, an attempt has been made to render an unkilled steel resistant to ageing by the addition of boron. Since, however, boron has a certain affinity to oxygen, the boron greatly reduces the boiling of the unkilled steel so that in this case too the resultant steel is impure. A procedure that has therefore been adopted is to hold up the introduction of the boron until a few minutes after pouring into the ingot, i.e., until a clean outer zone has already formed. Apart from the difficulty of distributing the boron in the ingot, this steel has been unsatisfactory for lack of purity of the ingot. Finally, an attempt was made to use partially killed steels. Since these steels have a low oxygen content, it was thought that oxidation of the boron could be prevented. Apart from insufficient purity, such attempts also resulted in considerable surface flaws, due mainly to the peripheral blow holes which are inevitable in a semi-killed steel and are situated just beneath the surface.

The object of the invention is to produce a deep-drawing steel which is resistant to ageing and has properties of Al-killed steel, under conditions which avoid the disadvantages of Al-killed steel and afford a very simple and economic production process.

To this end, according to the invention, the steel is tapped in an unkilled or partially killed state, its free oxygen is largely removed, for example down to a residual contact between 0.005% and 0.010% by weight, by degasification of batches in a vacuum chamber, and the oxygen remaining in the steel is further reduced by the addition of aluminum in an amount between 0.001% and 0.005% by weight, after which between 0.05 kg. and 0.10 kg. of boron per metric ton of steel is added to the steel (which is an addition of 0.005 to 0.10% by weight, of boron) and the steel thus treated is poured rapidly into an ingot mould at a rate of climb in the mould of 80 cm. per minute, preferably 120 cm. per minute.

The process is best carried out using steel with a carbon content of about 0.08%, and this steel is tapped into a ladle in an unkilled state from an open-hearth furnace and is then vacuum-treated in batches. During this degasification process, individual batches weighing about 10% of the ladle content are periodically drawn into the degasification chamber from the steel in the ladle through a pipe leading to the bottom of the degasification chamber and are returned through the same pipe to the

## 2

ladle after degasification. The degasification of each batch takes about 15–20 seconds.

An example of a process in accordance with the invention will now be described with reference to the accompanying drawings which show the apparatus used and in which:

FIG. 1 is a diagrammatic section through the apparatus at one stage of the process;

FIG. 2 is a similar section at a later stage;

FIGS. 3 and 4 are graphs showing the vacuum in the vacuum chamber during the process; and

FIG. 5 is a reproduction of an etched section of an ingot made by the process.

The apparatus comprises a degasification chamber 1 having a pipe 2 leading to its base, a ladle 3 filled with the melt for degasification, a connection 4 from the chamber to a vacuum pump and a tank 5 for introduction of treatment or alloying substances into the degasification chamber 1. In the position shown in FIG. 1, the pipe 2 dips into the charge in the ladle 3. In this position a batch of steel S is sucked into the tank where it is degasified. On raising the vacuum chamber to the position shown in FIG. 2 the degasified steel flows back through the pipe 2 into the ladle 3. This cycle of batch degasification is continued until the steel oxygen content has dropped to the required amount.

FIG. 3 shows the variation of the vacuum with time in the degasification chamber under these conditions. The abscissa of the diagram denotes time in minutes, and the ordinate vacuum pressure in torr (=mm. Hg). The vacuum, equal to about 50 torr at the beginning of the degasification operation, has dropped to about 5 torr after about 30 batch treatments. With a specifically dimensioned degasification chamber the pressure rise for a flow of equal batches into the tank is a measure of the free oxygen content of the steel. The relationship between the pressure rise of the batch entering the degasification vessel and the free oxygen content of the steel is determined from samples taken from the ladle during prior treatments.

The result is shown in FIG. 4, which refers to the pressure rise per metric ton of steel taken in. In this diagram the abscissa denotes pressure change per quantity in torr/t, and the ordinate denotes free oxygen content in  $\frac{1}{1000}$  by weight. From FIG. 4 it will be apparent that a pressure rise of 0.2 torr per metric ton of steel corresponds to a steel free oxygen content of 0.009% by weight. If it is required to degasify to this value the steel of a 100 metric ton ladle, 10 metric tons of steel being drawn in each batch, the degasification is continued until the pressure rise on entry of steel into the tank is equal to 2 torr. The pressure curve depends also on geometric conditions and the capacity of the suction apparatus used for the degasification plant. The conditions shown in FIG. 4 must therefore be determined empirically for each plant and each steel grade.

When the free oxygen content of the steel in the degasification chamber has dropped to the required value, preferably to between 0.005 and 0.010% by weight, aluminium is introduced via the vessel 5 into the batch in the degasification tank until the free quantity of oxygen in the charge in the ladle after the discharge of the batch has dropped to 0.001–0.005% by weight, preferably 0.003% by weight. The quantity of aluminium required for the purpose can be calculated correctly because there is no incalculable burning away when the aluminium is added via the discharge vessel. In the case described, the required final oxygen content in the molten steel was obtained by the addition of 70 grammes of aluminium per metric ton of steel. Boron was then added—again via the degasification chamber—the addition being made in the form of ferro-boron. To distribute the aluminium and boron uniformly in the charge it is preferable to draw in some more

batches of steel and return them to the ladle after the aluminium and boron have been added.

A melt prepared in this way was poured into moulds of a capacity of 15 metric tons each at a speed such that the moulds were full in about 1½ minutes. The ingot head was quenched with water.

FIG. 5 shows the nature of a steel treated in this way. It shows the structure of an ingot cut open longitudinally. It will be seen that the steel has no peripheral blow holes otherwise found in half-killed steels. The core structure of the metal is loosened to a certain extent but there is no unsatisfactory pipe formation.

The ageing-resistant deep-drawing steel prepared by the method according to the invention has no oxide inclusion in and beneath the surface of the ingots, such as are found in aluminium-killed steel. The steel can therefore be rolled very satisfactorily and rough slabbing gives a surface quality such that no flame descaling is required. Another advantage of the steel is the high and uniform yield due to its favorable solidification structure. For example, an average yield of 93.5% was obtained for a charge, and varied only between 93 and 94% in the individual ingots.

I claim:

1. A process for the manufacture of deep-drawing steel which is resistant to ageing comprising the steps of tapping said steel in an at least partially unskilled state, degasifying said tapped steel in batches in a vacuum chamber to largely remove the free oxygen therefrom, adding aluminium to said steel to reduce its oxygen content further to between 0.001% and 0.005% by weight, adding between 0.05 kg. and 0.10 kg. of boron per metric ton of steel to said steel and pouring said steel rapidly into an ingot mould at a rate of climb in said mould of at least 80 cm. per minute.

80 cm. per minute.

2. A process as claimed in claim 1, in which said degasifying step is carried out until said free oxygen is reduced to a value of between 0.005% and 0.01% by weight of said steel.

of said steel.

3. A process as claimed in claim 1, in which said pouring step takes place at a rate of climb in said mould of 120 cm. per minute.

4. The method of producing non-aging steels comprising the steps of subjecting a molten steel bath to a vacuum sufficient to cause removal of oxygen from the bath, maintaining the bath under vacuum until the oxygen level in

lanning the bath under vacuum until the oxygen level in

the bath is reduced to about 0.005% to about 0.01%, adding aluminium to the steel in an amount sufficient to react with the remaining oxygen to reduce the oxygen level below about 0.003% and adding 0.005% to 0.010% boron to the molten bath following the aluminium addition.

5        5. The method of producing non-aging steels comprising  
the steps of subjecting a molten steel bath to a vacuum  
sufficient to cause removal of oxygen from the bath, main-  
taining the bath under vacuum until an oxygen level below  
about 0.01% is attained in the steel, adding an amount  
10      of aluminium to the steel sufficient to reduce the oxygen  
level below about 0.003% and adding about 0.005 to  
0.010% boron to the molten bath following the aluminium  
addition.

15 addition. 6. The method of producing non-aging steels comprising the steps of subjecting a molten steel bath to a vacuum sufficient to cause removal of oxygen from the bath, maintaining the bath under vacuum until the oxygen level is reduced to about 0.005% to about 0.010%, adding an amount of aluminium sufficient to react with the remaining oxygen to reduce the oxygen level below about 0.003%, and thereafter adding about 0.005 to 0.010% boron to the molten bath.

25      7. The process of preparing a non-aging steel comprising  
the steps of subjecting a molten bath of steel containing  
about 0.08% carbon to a vacuum sufficient to cause  
removal of oxygen from the bath, maintaining the bath  
under a vacuum until the oxygen level in the bath is re-  
duced to about 0.005% to about 0.01%, adding alumin-  
30      ium to the steel to react with the remaining oxygen to  
reduce the level of oxygen below about 0.003%, adding  
about 0.005% to 0.10% of boron to the molten bath and  
casting the resulting molten bath.

### References Cited

UNITED STATES PATENTS

- |           |         |               |       |     |   |    |   |
|-----------|---------|---------------|-------|-----|---|----|---|
| 2,768,892 | 10/1956 | Shoenberger   | ----- | 164 | — | 57 | X |
| 3,183,078 | 5/1965  | Ohtake et al. | ----- | 75  | — | 49 |   |
| 3,208,844 | 9/1965  | Kato et al.   | ----- | 75  | — | 49 |   |

HENRY W. TARRING II, Primary Examiner

U.S. CL. X.R.

15 75-129; 164-57, 133